

Sept. 6, 1932.

C. L. MORRIS

1,876,015

PROCESS OF GLAZING ARTIFICIAL TEETH

Filed Feb. 28, 1929



Fig. 3.



Fig. 2.

Inventor  
Charles Leon Morris

By George S. Garside

Attorney

## UNITED STATES PATENT OFFICE

CHARLES LEON MORRIS, OF COLUMBUS, OHIO, ASSIGNOR TO THE COLUMBUS DENTAL MANUFACTURING COMPANY, OF COLUMBUS, OHIO, A CORPORATION

## PROCESS OF GLAZING ARTIFICIAL TEETH

Application filed February 28, 1929. Serial No. 343,504.

The object of this invention primarily applies to the dental art and the object is to provide a method and a means that will effectively and efficiently bake, glaze and stain artificial teeth.

Another important object of this invention is to provide a much more economical method than has been previously employed.

Another important object of this invention is to provide a proper cooling and annealing treatment.

In the drawing:

Figure 1 is a perspective view of a glazing furnace.

Figure 2 is a perspective view of a tray and cover.

Figure 3 is a perspective view of the tray.

Figure 4 is a longitudinal sectional view of the tray and cover.

Another important object is to provide a means whereby artificial teeth may be protected against specks or blemishes while being baked, glazed, stained or annealed.

The reference numeral 5 designates a furnace of suitable construction for carrying out my method of glazing dental porcelain, said furnace having a suitable closure 6.

In carrying out my method of glazing dental porcelain I use a thin refractory slab or base 7 having preferably, a seat 8 in its upper face and extending entirely around the slab within the outer edge of the slab, in which is seated the lower edge of a cover 9 also made thin and refractory.

The slab and cover are made of material having high heat conductivity properties and presents very little temperature lag which results in the heat intensity exerted on the enclosed ware (dental porcelain) registering substantially the same as the heat intensity immediately surrounding the refractory cover.

The cup or depression X in the cover is designed to hold a certain amount of gold. One may by looking through a peep hole in the

kiln observe the state of the gold from time to time, and when the gold has become molten the operator knows that the glazing of the dental porcelain is finished.

The improved method practiced in carrying out this invention consists in employing an electric resistance furnace having a nickel chromium element directly exposed, and in order to protect the ware from the objectional particles caused by spalling, a small, thin refractory cover has been designed, which latter is inverted over the ware. The thin refractory cover is composed of material having high heat conductivity properties and presents very little temperature lag which results in the heat intensity exerted on the enclosed ware registering substantially the same as the heat intensity immediately surrounding the refractory cover.

This method further comprehends the simultaneous conveying of the ware and cover into and out of the furnace, so that the ware is at no time directly exposed to the detrimental spalling action of the heating element. The refractory cover in its broadest sense preferably comprehends two parts, namely, a thin slab or base portion and a cover portion proper. It may be thought of as a small removable muffle completely enclosing the ware. In applying this method the ware is first placed on the thin refractory slab, or base, while the latter is outside of the furnace chamber. The refractory cover is then placed over the ware and all parts are simultaneously conveyed into the heat chamber where the ware receives the proper heat treatment. After the ware has had sufficient heat treatment imposed upon it, the base, cover and ware are simultaneously removed, the ware thus remaining covered and protected.

This method further comprehends a rapid, yet safe, cooling and annealing period for the ware. It is common knowledge that ceramic ware can be cooled too rapidly, which latter action promotes crystallization of the ware.

and causes it to be weak and fragile structurally. In the past it has been common practice to slowly cool and anneal the ware in the furnace chamber proper. This method is somewhat slow and renders the furnace chamber useless for the introduction of new ware.

Another method of cooling and annealing, which consists in having a separate chamber for cooling, has been employed. This necessitates an extra amount of equipment and is not entirely satisfactory because the chamber is usually at room temperature, which often imposes a shock or chill, to the ware, until the heat radiation of the ware itself has raised the temperature within the chamber to relatively near that of the rapidly cooling ware. In other words, the ware is cooled too rapidly during its first annealing period. In my improved method the ware is cooled at an even rate, yet efficiently and rapidly, due to the high heat conductivity property of the cover and base, and the ware is thoroughly protected from direct exposure to the atmosphere of the room thus annealing it properly and adding materially to its strength. This method thus avoids the weakness and fragility due to improper cooling methods.

This method comprehends the use of several removable muffles, which latter are not expensive, and allows the operator to proceed with new ware to the furnace without a decided heat halt between heat treatments.

This improved method has a further advantage over the methods used in the past in that the repair of the furnace is comparatively inexpensive. It can readily be seen that when a platinum resistance element burns out that the repair expense of such a furnace will be considerable in excess of the repair expense in replacing with a new heating element composed of nickel chromium.

In applying the improved method it has been found that the life of the resistance heating element of nickel chromium is equal to, and in some instances greater than, the life of the platinum resistance element: that is to say, the nickel chromium resistance element will stand as much, or more, service than the platinum resistance element at their respective service temperatures.

What I claim is:

The method of glazing artificial teeth in an electrical resistance furnace employing a resistor exposed in the furnace chamber so as to protect the tooth against spalling from the resistor and from injury by atmospheric impurities or too sudden cooling after glazing, which method consists in enclosing the tooth in a covered dust-proof receptacle of refractory material sufficiently thin to allow ready passage of heat therethrough and sufficiently refractory to withstand the operating temperature of the furnace, disposing the receptacle in the furnace chamber and subjecting it

therein while the tooth is excluded thereby from direct exposure to the atmosphere of said chamber to the action of heat of sufficient temperature and for a sufficient period of time to glaze the tooth, and removing the receptacle from the furnace and allowing it to freely cool to the temperature of the air while the cover is applied so as to protect the tooth from exposure to the air while cooling.

In testimony whereof I affix my signature.

CHARLES L. MORRIS.

80

85

90

95

100

105

110

115

120

125

130